# EUROPEAN PATENT SPECIFICATION

(11) **EP 0 192 703 B1**
(45) Date of publication and mention of the grant of the patent: **02.11.1989**
(21) Application number: 85904351.5
(22) Date of filing: 19.08.1985
(51) Int. Cl.: H01H 1/02

(54) **NICKEL-BASED ELECTRICAL CONTACT**
ELEKTRISCHER KONTAKT AUF NICKELBASIS
CONTACT ELECTRIQUE A BASE DE NICKEL

(30) Priority: 31.08.1984 US 646707; 01.08.1985 US 761402
(43) Date of publication of application: 03.09.1986
(73) Proprietor: AT&T Corp., New York, NY 10013-2412 (US)
(72) Inventor: HAUSER, Joachim, Jacques, Summit, NJ 07901 (US); PLEWES, John, Travis, Chatham, NJ 07928 (US); ROBBINS, Murray, Berkeley Heights, NJ 07922 (US)
(74) Representative: Johnston, Kenneth Graham
(86) International application number: US8501587
(87) International publication number: WO8601636

(56) References cited:
- DE-A- 1 945 592
- FR-A- 2 211 536
- FR-A- 2 293 042
- US-A- 1 769 229
- US-A- 3 017 532

## Description

### Technical field

The invention is concerned with electrical contact surfaces and, more specifically, with nickel- based contact surface materials.

### Background of the invention

Typically, the manufacture of high-quality electrical contacts has involved the use of gold whose properties of low contact resistance and high chemical stability are key advantages in such usage. However, as the price of gold remains high, efforts continue at finding alternative materials for contact manufacture.

Prominent among such alternatives are precious metals other than gold; e.g. silver-palladium alloys have been found suitable for certain applications. While such alternate alloys are less expensive than gold, still further cost reduction is desired, and nonprecious metal alloys such as, e.g. copper-nickel alloys have also been investigated for contact resistance and stability overtime. See S. M. Garte et al. "Contact Properties of Nickel-Containing Alloys", Electrical Contacts, 1972, Illinois Institute of Technology.

U.S. Patents 1,769,229 and 3,017,532 are directed to electrodes and contact elements subject to electric arcs, each contact comprising a substantial amount of nickel and at least one additional element.

According to the present invention there is provided apparatus as defined in claim 1. It has been discovered that certain nickel alloys have contact properties of high stability and low contact resistance comparable to those of gold. Devices in accordance with the invention comprise a contact surface which is the surface of such alloy comprising nickel and at least one glass-forming additional element such as boron, silicon, germanium, phosphorus, arsenic, antimony, or bismuth. The presence of such glass-forming element is considered to inhibit the formation of semiconducting nickel oxide and/orto result in the formation of a thermodynamically more stable compound, preserving metallic conductivity of a contact layer in an oxidizing ambient.

The addition of one or several glass-forming elements results in a crystallographically disordered structure at least upon exposure of the layer to an oxidizing ambient, this as contrasted with the formation of crystalline nickel oxide in the absence of preferred addition of a glass-forming element. Alternatively, crystallographically disordered structure can be produced by ion bombardment, alpha particles being conveniently used for this purpose.

Surface contact resistance less than 100 milliohms is typically maintained even after prolonged exposure to an oxidizing ambient.

### Brief description of the drawing

Fig. 1 is a perspective view of an electrical connector device in accordance with the invention; and
Fig. 2 is a schematic cross-sectional view of a portion of a device in accordance with the invention.

### Detailed description

The electrical connector device shown in Fig. 1 comprises housing 11 and contact pins 12. Housing 11 is made of an electrically insulating material, and contact pins 12 have contact surfaces in accordance with the invention.

Shown in Fig. 2 are, in cross section, an electrically conducting member 21 on which a surface layer 22 is situated. In accordance with the invention surface layer 22 is made of an alloy of nickel and at least one glass-forming additional element. Upon exposure to an oxidizing atmosphere, portion 23 of layer 22 further comprises oxygen.

Preferred glass-forming additive elements are boron, silicon, germanium, phosphorus, arsenic, antimony, and bismuth, and their presence in the contact layer is in a preferred amount in the range of from 1 to 40 and preferably 2 to 10 atom percent relative to the combined amount of nickel and the additive element; preferred also in the range of from 25 to 35 atom percent where thermodynamically stable, stoichiometric compounds are formed.

In combination, nickel and the glass-forming additive element or elements constitute a preferred amount of at least 70 atom percent of the contact layer material. In the interest of enhanced electrically and mechanical contact properties, the addition of cobalt is desirable, elements otherthan cobalt preferably being limited to amounts less than 5 atom percent in combination and preferably less than 1 atom percent. Particularly undesirable is the presence of Group VI elements such as sulfur, selenium, and tellurium, and their combined amount is preferably limited to less than 0.5 atom percent.

In the case of non-stoichiometric aggregates, glass-forming additives to nickel are considered to inhibit the formation of semiconducting nickel oxide in an oxidizing ambient. Instead of such semiconducting nickel oxide, in the presence of the glass-forming additive, a surface layer of an aggregation including nickel, oxygen, and the glass-forming additive is believed to be formed in sufficiently large regions of the layer, such aggregation having essentially metallic conduction properties. Based on experimental evidence the thickness of the oxygen-containing surface layer is estimated to be on the order of 2.5 nm.

Crystallographically disordered structure in nickel-containing layers is produced also upon ion bombardment which results in a crystallographically disordered structure even before exposure to an oxidizing ambient. Still, it is the disordered, quasi-amorphous, glass-like nature of an oxidized surface portion which is considered to be conducive to desired low contact resistance of a contact layer for use in an oxidizing ambient. A crystallographically disordered nickel aggregate preferably comprises nickel in an amount of at least 50 atom percent.

The following examples specifically illustrate the suitability of contacts in accordance with the invention.

### Example 1

A layer consisting essentially of 95 atomic percent nickel and 5 atomic percent antimony was deposited by getter-sputtering approximately 3 micrometers thick on a copper substrate. Standard four-point probes were used to determine surface contact resistance; such resistance was found to be in the range of from 5 to 7 milliohms. The deposited film was then subjected to a test for stability at elevated temperature and humidity (65 hours at a temperature of 75 degrees C, relative humidity of 95 percent), and contact resistance was then found to be in the range of from 15 to 20 milliohms.

### Example 2

An experiment was carried out, analogous to Example 1, on a layer consisting essentially of 95 atomic percent nickel and 5 atomic percent phosphorus. Contact resistance was 1.8 milliohm before the test and 4.4 to 5 milliohms after the test.

### Example 3

An experiment was carried out, analogous to Example 1, on a layer consisting essentially of 95 atomic percent nickel and 5 atomic percent boron. Contact resistance was in the range of from 2.9 to 3.5 milliohms before the test and in the range of from 10 to 14 milliohms after the test.

### Example 4

An experiment was carried out, analogous to Example 1, on a layer consisting essentially of 95 atomic percent nickel and 5 atomic percent silicon. Contact resistance was in the range of from 1.6 to 2.1 milliohms before the test and in the range of from 4.5 to 6 milliohms after the test.

### Example 5

An experiment was carried out, analogous to Example 1, on a layer consisting essentially of 95 atomic percent nickel and 5 atomic percent germanium. Contact resistance was in the range of from 1.5 to 1.85 milliohms before the test and 10 to 14 milliohms after the test.

### Example 6

An aqueous solution was prepared containing 208 gm/I NiCl₂ . 6H₂0, 49 gm/I H₃P0₄ 85 percent, and 5 gmll H₃P0₃. The solution was used to electroplate onto a copper electrode; plating bath temperature was 75 degrees C, current density was 150 mA/cm², and plating rate was approximately 3 micrometers per minute. The deposited layer had a thickness of approximately 4.5 micrometers. Contact resistance of the deposited layer was less than 10 milliohms after exposure to the testing ambient.

### Example 7

An aqueous solution of 0.087 molar of As₂O₅ and 0.5 molar of NiCI₂. 6H₂0 was prepared. A copper electrode was plated with nickel arsenide by pulse-plating from the solution at a temperature of 75 degrees C; current pulses of 200 mA/ cm² were on for 1.5 seconds and off for 0.5 seconds. Deposited layer thickness was approximately 4.5 micrometers. Contact resistance of the deposited layer was less than 10 milliohms after exposure to the testing ambient.

### Example 8

To a solution of 5 gm Ge0₂ in 50 cc water plus 4 cc ammonium hydroxide and 0.5 molar of NiC-I₂ . 6H20,150 gm/1 ammonium citrate were added. The solution was filtered, and ammonium hydroxide was added until pH was 8.5. A layer of nickel-germanium was plated from the solution at a temperature of 75 degrees C onto a copper electrode; current density was 150 mA/cm² and plating rate was approximately 2.5 micrometers per minute. Deposited layer thickness was approximately 4.5 micrometers. Contact resistance of the deposited layer was less than 10 milliohms after exposure to the testing ambient.

### Example 9

A layer of nickel having a thickness of approximately 350 nm was deposited on a polished copper foil. A portion of the nickel layer was covered with an aluminum foil, and alpha-particles were implanted in the uncovered portion of the nickel layer. Alpha-particles had an energy of approximately 1.8 MeV, and a dose of approximately 1.6×10¹⁶ particles per cm² was found to be optimal or near-optimal for minimized contact resistance (less than 10 milliohms) after exposure to humid air at elevated temperature as described in Example 1 above. (This test is considered to be an approximate equivalent of exposure to ordinary atmospheric conditions for a duration of 5 years). Also, visual inspection of the implanted portion after the test as compared with the portion which had been covered with aluminum foil, showed the latter to be dull and brownish while the former appeared bright and shiny.

## Claims

1. Apparatus comprising an electrical contact, said contact (12) comprising a body of contact material (22) which comprises a substantial amount of nickel and at least one additional element, characterized in that said at least one additional element is a glass forming element selected from boron, silicon, germanium, phosphorus, arsenic, antimony, and bismuth, said at least one additional element being present in said contact material in an amount in the range of from 2 to 10 atom percent of the combined amount of nickel and said at least one additional element, said combined amount being greater than or equal to 70 atom percent of said contact material, and at least a surface portion (23) of said

body of contact material has a crystallographically disordered structure produced upon exposure of - said contact material to an oxidizing ambient or by ion bombardment, said surface portion having a relatively low contact resistance.

2. Apparatus of claim 1, characterized in that said body of contact material being in the form of a layer deposited on a substrate (21).

3. Apparatus according to claim 1 or 2, characterized in that said surface portion having a contact resistance which is less than 100 milliohms.

4. Apparatus according to claim 1 or 2 or 3, characterized in that said contact material further comprises cobalt.

5. Apparatus according to any one of preceding claims 1-4, characterized in that said contact material comprises at least 50 atom percent nickel and said disordered structure is produced by ion bombardment.

6. Apparatus according to any one of preceding claims 1-5, characterized in that the presence of sulfur, selenium, and tellurium in combination is limited in said contact material to less than 0.5 atomic percent.

7. Apparatus according to any one of preceding claims 1-6, characterized in that said at least one additional element being boron or phosphorus or arsenic.

8. Apparatus according to any one of preceding claims 1-6, characterized in that said at least one additional element being silicon or germanium.

9. Apparatus according to any one of preceding claims 1-6, characterized in that said at least one additional element being antimony or bismuth.

## Patentansprüche

1. Vorrichtung mit einem elektrischen Kontakt, wobei der Kontakt (12) einen Körper aus Kontaktmaterial (22) umfaßt, der einen wesentlichen Nickelanteil und wenigstens ein zusätzliches Element enthält, dadurch gekennzeichnet, daß
das zusätzliche Element ein glasbildendes Element ist, das von Bor, Silicium, Germanium, Phosphor, Arsen, Antimon und Wismuth ausgewählt ist,
das zusätzliche Element in dem Kontaktmaterial in einem Anteil von 2 bis 10 Atom-%, bezogen auf den kombinierten Anteil von Nickel und zusätzlichem Element, vorhanden ist, wobei der kombinierte Anteil größer oder gleich 70 Atom-% des Kontaktmaterials ist, und
wenigstens ein Oberflächenteil (23) des Kontaktmaterialkörpers eine kristallographisch ungeordnete Struktur besitzt, die durch Aussetzen des Kontaktmaterials einer oxidierenden Umgebung oder durch Ionenbombardement erzeugt ist, wobei der Oberflächenteil einen relativ niedrigen Kontaktwiderstand besitzt.

2. Vorrichtung nach Anspruch 1, dadurch gekennzeichnet, daß der Kontaktmaterialkörper in Form einer auf ein Substrat (21) niedergeschlagenen Schicht ist.

3. Vorrichtung nach Anspruch 1 oder 2, dadurch gekennzeichnet, daß der Oberflächenteil einen Kontaktwiderstand von weniger als 100 Milliohm besitzt.

4. Vorrichtung nach Anspruch 1, 2 oder 3, dadurch gekennzeichnet, daß das Kontaktmaterial des weiteren Cobalt umfaßt.

5. Vorrichtung nach einem der vorstehenden Ansprüche 1 bis 4, dadurch gekennzeichnet, daß das Kontaktmaterial wenigstens 50 Atom-% Nickel umfaßt und die ungeordnete Struktur durch lonenbombardement erzeugt wird.

6. Vorrichtung nach einem der vorstehenden Ansprüche 1 bis 5, dadurch gekennzeichnet, daß die Gegenwart von Schwefel, Selen und Tellur in dem Kontaktmaterial zusammengenommen begrenzt ist auf weniger als 0,5 Atom-%.

7. Vorrichtung nach einem der vorstehenden Ansprüche 1 bis 6, dadurch gekennzeichnet, daß das zusätzliche Element Bor oder Phosphor oder Arsen ist.

8. Vorrichtung nach einem der vorstehenden Ansprüche 1 bis 6, dadurch gekennzeichnet, daß das zusätzliche Element Silicium oder Germanium ist.

9. Vorrichtung nach einem der vorstehenden Ansprüche 1 bis 6, dadurch gekennzeichnet, daß das zusätzliche Element Antimon oder Wismuth ist.

## Revendications

1. Dispositif comprenant un contact électrique, ce contact (12) comprenant une partie qui consiste en un matériau de contact (22) qui contient une quantité notable de nickel et au moins un élément supplémentaire, caractérisé en ce que le ou les éléments supplémentaires consistent en éléments formant un verre, sélectionnés parmi le bore, le silicium, le germanium, le phosphore, l'arsenic, l'antimoine et le bismuth, le ou les éléments supplémentaires sont présents dans le matériau de contact en une proportion, en pourcentage atomique, dans la plage de 2 à 10% de la quantité combinée de nickel et de l'élément ou des éléments supplémentaires, cette quantité combinée étant supérieure ou égale à un pourcentage atomique de 70% du matériau de contact, et au moins une région de surface (23) de la partie de matériau de contact à une structure désordonnée au point de vue cristallographique, qui est produite sous l'effet de l'exposition du matériau de contact à une ambiance oxydante ou par bombardement ionique, cette région de surface ayant une résistance de contact relativement faible.

2. Dispositif selon la revendication 1, caractérisé en ce que la partie de matériau de contact se présente sous la forme d'une couche déposée sur un substrat (21).

3. Dispositif selon la revendication 1 ou 2, caractérisé en ce que la région de surface a une résistance de contact qui est inférieure à 100 milliohms.

4. Dispositif selon la revendication 1, 2 ou 3, caractérisé en ce que le matériau de contact comprend en outré du cobalt.

5. Dispositif selon l'une quelconque des revendications 1 à 4 précédentes, caractérisé en ce que le matériau de contact comprend un pourcentage atomique d'au moins 50% de nickel, et la structure désordonnée est produite par bombardement ionique.

6. Dispositif selon l'une quelconque des revendications 1 à 5 précédentes, caractérisé en ce que la quantité de soufre, de sélénium et de tellur, en combinaison, est limitée dans le matériau de contact à un pourcentage atomique inférieur à 0,5%.

7. Dispositif selon l'une quelconque des revendications 1 à 6 précédentes, caractérisé en ce que le ou les éléments supplémentaires consistent en bore, en phosphore ou en arsenic.

8. Dispositif selon l'une quelconque des revendications 1 à 6 précédentes, caractérisé en ce que le ou les éléments supplémentaires consistent un silicium ou en germanium.

9. Dispositif selon l'une quelconque des revendications 1 à 6 précédentes, caractérisé en ce que le ou les éléments supplémentaires consistent en antimoine ou en bismuth.
